

## UNITED STATES PATENT OFFICE

2,292,541

ACCELERATION OF THE SEASONING SPEED  
OF SURFACE COVERINGSDonald G. Patterson, Stamford, Conn., assignor to  
American Cyanamid Company, New York,  
N. Y., a corporation of MaineNo Drawing. Application April 26, 1940,  
Serial No. 331,811

## 1 Claim. (Cl. 106—264)

This invention relates to the acceleration of the rate of curing or "seasoning" of surface covering compositions such as floor covering compositions containing siccative binders.

An object of this invention is to provide accelerators for surface covering compositions containing siccative binders which will cause such compositions to cure more rapidly.

This and other objects are attained by incorporating in a siccative composition which is to be used in a floor covering composition or other surface covering composition formoguanamine.

The following example is given by way of illustration and not in limitation.

## Example

|                  | Parts by weight |
|------------------|-----------------|
| Siccative binder | 30              |
| Wood flour       | 30              |
| Whiting          | 20              |
| Lithopone        | 20              |
| Formoguanamine   | 0.1             |

These substances with or without a small proportion of drier, e. g., 0.1% cobalt naphthenate, are mixed together, e. g., in an internal mixer. The compacted mass which is delivered from the mixer may be disintegrated, as by a set of "scratch rolls" which comprises a plurality of rolls having intermeshing teeth projecting from their surfaces. The resulting material is sheeted on calender rolls or optionally it may be further mixed and disintegrated and then calendered. The material may be calendered on to burlap or other fibrous backing if desired. The sheeted material is placed in a stoving oven through which a current of heated air from about 70° C. to about 90° C. is circulated until the material is completely "seasoned", i. e., until the sheet acquires the necessary degree of hardness. Higher or lower temperatures may be used if desirable.

The hardness may be measured by any of the methods generally employed in the manufacture of linoleum. See the Federal Stock Catalogue (U. S. Government Printing Office), section 4, part 5, pages LLL-L-351 et seq. and pages LLL-L-361 et seq., for the method employed herein. The time required for "seasoning" a 2 mm. sheet of the above composition is about 4 to 5 days. The resulting "seasoned" floor or surface covering has about the same strength, flexibility and color as compositions not containing the accelerator. One or more of these properties may be changed by many other accelerators sufficiently and in such a way that the materials

produced therewith are unsatisfactory. The "seasoning speed" of a 2 mm. sheet of the same mixture which does not contain the formoguanamine is about 18 to 20 days.

5 The siccative binder utilized in the above example is an alkyd resin which has siccative properties, i. e., a reaction product of fumaric acid with a non-conjugated terpene (alpha pinene) and triethylene glycol, modified with linseed oil fatty acids. Other similar resins may be used which are drying oil-modified reaction products of maleic or fumaric acids with a terpene and a polyhydric alcohol. Other alkyd resins which are modified with drying oils may be used such as 10 the phthalic-glyceride resins, the glycol-maleic resins, and mixed resins such as the phthalic-fumaric-glycol-glyceride resins. With other types of binders, the "seasoning" temperature may be varied appropriately and, of course, the time required may be different. About the same proportional accelerating effect is obtained when various siccative binders are employed.

Other binders which may be used are those which are derived from the drying oils and may be made in any convenient well-known manner, such as the method described in British Patent 305,656, or the binders may comprise any of the various alkyd resins having siccative properties. For drying oil binders, linseed oil is preferable 20 for economic reasons, but other siccative oils may be used such as, for example, menhaden or fish oil, tung oil, soya-bean oil, perilla oil, oiticica oil, Scheiber oil, sunflower-seed oil, etc. The term "siccative oil" as used herein is intended to include not only the so-called drying oils but also the so-called semi-drying oils. Furthermore, it is possible to use mixtures of siccative oils with other fatty oils of the non-drying type.

It may be preferable in the manufacture of 25 linoleum to make use of so-called "scrim-oil" or "shed oil" either alone or fluxed with rosin or other gums or resins and/or mixed with a proportion of the so-called "mechanical oil." Either of these types of oils may be used singly if desired.

In the preparation of the siccative oil binders it is customary to use rosin in admixture with the oil although other substances of the same type may be used, e. g., Kauri gum, Congo gum, ester gum, abietic acid and its esters, pimamic acid, etc.

Instead of wood flour and/or the whiting and lithopone used in the example, other fillers or pigments may be used. Examples of such fillers are: cork, cellulose pulp, asbestos, cottonwood tree pulp, walnut shell meal, glass fibers, foliated

glass, etc. Among the pigments which may be used the following are included: lithopone, barytes, zinc oxide, titanium oxide, chromates, red lead, white lead, malachite green, chrome green, chrome yellow, Prussian blue, iron oxide, etc. Similarly dyes and lakes may be used if desirable.

It is generally preferable to use driers in the preparation of the binders. The drier is usually added to the binder during the oxidation process and if desirable additional drier may be added when the binder, fillers, etc., are mixed together. Suitable driers include the oil-soluble salts such as the naphthenates, resinates and linoleates of cobalt, lead, manganese, zinc and chromium. Only a small proportion of these driers based on the siccative oil content is generally sufficient, e. g., about 0.005-1%, although larger proportions may be used as expedient. Obviously, various mixtures of driers may be used.

The term "seasoning" as applied to linoleum compositions indicates the process of curing by heating or equivalent treatment to polymerize and/or oxidize the composition to a stage where-in the floor covering is sufficiently hard and resistant to abrasion to be suitable for its intended purpose and yet is still sufficiently flexible to permit the usual bending and rolling required of linoleum. The term "maturing" is similarly used.

I have found that only a small proportion of formoguanamine is generally sufficient, e. g., 0.1-5% of the siccative composition but obviously smaller or larger proportions may be used if desirable. In some instances, the alkali resistance may be improved somewhat by the use of formoguanamine.

My accelerator is preferably added during the mixing of the binder with the fillers, etc., although it may be added before or during the oxidation of the binder. If my accelerator is added before or during the oxidation, it may inhibit somewhat the gelation of the siccative binder. It is to be noted, however, that after gelation, my accelerator speeds up the curing of the siccative composition.

Obviously many modifications in the processes and compositions described above may be made without departing from the spirit and scope of the invention as defined in the appended claim.

I claim:

In a process of curing a surface covering composition including a siccative material selected from the group consisting of drying oils and drying oil modified polyhydric alcohol-polybasic acid resins, the step which comprises adding to such a composition formoguanamine.

DONALD G. PATTERSON.